

## UNITED STATES PATENT OFFICE

2,655,148

ADHESIVE FOR PLASTER OF PARIS FOR  
BANDAGE USEJames Joseph Eberl, Chester, and Alvin Richard  
Ingram, Glenshaw, Pa., assignors to Johnson  
& Johnson, a corporation of New JerseyNo Drawing. Application February 1, 1950,  
Serial No. 141,848

11 Claims. (Cl. 128—91)

1

This invention relates to a bandage for use in surgery, orthopedics and dermatology, and particularly one of the type wherein a flexible fibrous carrier is impregnated with a composition containing plaster of Paris together with an adhesive binder to prevent plaster loss.

Such a bandage is made usually in the form of a roll which, in use, is immersed in water to hydrate the plaster and, while still wet, wrapped around the member to be immobilized. During the wrapping process the bandage is molded to the shape of the member and rendered substantially homogeneous throughout by rubbing or handling. The bandage sets to form a hard and rigid structure.

Plaster of Paris bandages, as heretofore made, have not been entirely satisfactory. They sometimes lose as much as twenty-five per cent of the plaster during the immersion process and during application to the member to be immobilized. They require great care in handling to guard against telescoping, i. e., the tendency for the inner convolutions of the bandage to slip from within the outer convolutions as the bandage becomes thoroughly wetted. Where telescoping occurs, it is impossible to use a bandage in the manner intended.

In the improved bandage, telescoping, for all practical purposes, has been eliminated. It is unnecessary to use special precautionary techniques to guard against inter-layer slippage during immersion to saturate the bandage prior to use. During immersion, little or no plaster is lost and this is likewise true when the bandage is squeezed to expel excess water. The tests have shown that during the immersion and squeezing process the plaster lost from the improved bandage is in the neighborhood of 0.1%. It is true that as the bandage is molded on the member to be immobilized some plaster comes off on the operator's hands but this amounts to no more than about 3 to 5% of the total plaster in the bandage. Thus, about 94 to 96% of the original plaster in the bandage is delivered to the cast. The result is that more plaster per bandage is carried to the cast and fewer bandages are required for strong, dependable immobilization. To state the matter differently, bandages which initially contain a given amount of plaster produce a much stronger cast than earlier types of bandages containing initially a corresponding amount of plaster because of the excessive plaster loss suffered by the latter during application.

According to the present invention, the plaster of Paris (calcium sulfate hemi-hydrate) is held

2

in place on the flexible carrier prior to use by an adhesive which is insoluble in water or at least insoluble to such an extent as not to swell or otherwise be affected materially in the period required to wet-out the plaster. The adhesive is not present in the form of a film as in the case of the soluble adhesives that have heretofore been used, but rather is dispersed intermittently in the form of tiny discrete particles over the surface of the plaster particles binding them one to another and to the flexible carrier.

It has been discovered that the effect of the adhesive, in reducing plaster loss during the immersion process and eliminating telescoping during application to the member to be immobilized due to poor lamination, is governed by the quantity of adhesive used. Plaster of Paris bandages containing an adhesive, based on dry weight, in an amount within the range of from 0.1% to 2.5%, based on the dry weight of plaster of Paris, exhibit excellent laminating properties and, when used in the immobilization of body members, deliver to the cast approximately 94 to 96% of the original plaster in the bandage.

25 In the absence of a film or matrix in which the plaster of Paris particles otherwise would be embedded, there is nothing to delay or inhibit hydration when the bandage is immersed since during immersion the water will have immediate access 30 to the hemi-hydrate particles. Furthermore, throughout the immersion process, the insoluble, or relatively insoluble discrete particles of adhesive will continue to perform their binding function. They enable excess water to be 35 squeezed out without plaster loss so that the bandage will set and dry in the shortest possible period. Less adhesive is required than is the case if a continuous water soluble film is used.

In order to distinguish as a class the adhesive 40 materials it is proposed to use, they have been termed, in the absence of a better name, "non-swelling" adhesives and they may be either insoluble in water or so slowly soluble in water as not to swell during the period of wetting out and application of the bandage as previously described. Among the materials in this category which may be used in practising the invention there are included the water insoluble polymers and copolymers of vinyl acetate and methacrylate or acrylate esters; water insoluble cellulosic ethers and esters; natural and synthetic rubbers; coumarone indene resins; rosins and those derivatives of rosin which are water insoluble. These materials are given by way of example only since, 45 indeed, any adhesive which is water insoluble to

the extent previously mentioned may be used so long as it may exist in the form of an emulsion or dispersion which is stable under the conditions that exist during impregnation of the flexible carrier with the plaster of Paris.

Several methods may be used to incorporate the non-swellable adhesive in the plaster of Paris in the form of tiny discrete particles. One method is analogous to the acetic acid process described in the Mathey Patent 1,726,403, except that the non-swellable adhesive is a high viscosity water insoluble polyvinyl acetate which is introduced in the form of an emulsion. A suitable polyvinyl acetate emulsion for the purpose is obtainable in this country from E. I. du Pont de Nemours under the name "Elvacet 81A-900." This emulsion contains 55% by weight of polyvinyl acetate in water. For best results its viscosity in acetic acid (1 part emulsion to 9 parts glacial acetic acid by weight) should range between 300 to 2800 centipoises. This entire range is satisfactory but most efficient results are obtainable within the range 700 to 2000 centipoises. Below this range the adhesive suffers somewhat in adequacy, whereas above the range the polyvinyl acetate is not as effectively softened by the acetic acid, with the result that some of its adhesive action is lost. However, any disadvantages that might result from using the lower or the higher range may be compensated for by increasing the amount of emulsion per unit weight of plaster of Paris.

Particle fineness in the emulsion will be satisfactory if there is no significant settling out of the larger particles within 5 minutes after agitation of a mixture of 1 pint of the emulsion to 25 pints of water.

To prepare a suitable bandage, a batch of material using the polyvinyl acetate emulsion described above may be made up according to the following example:

#### Example I

|                            |       |             |
|----------------------------|-------|-------------|
| Plaster of Paris           | lbs.. | 200         |
| Water                      | lbs.. | 56          |
| Acetate acid (45%)         | lbs.. | 46          |
| Polyvinyl acetate emulsion | ml.   | 600 to 1800 |

The polyvinyl acetate emulsion is added to the water and the mixture agitated until complete dispersion is obtained. The dispersed emulsion is added slowly to the acetic acid while the latter is stirred. After two minutes stirring, the plaster of Paris is added in powdered state and the stirring continued until a smooth creamy slurry results. The slurry is spread on gauze, crinoline or other flexible carrier and then dried in any approved manner.

The amount of water and acetic acid used may be varied from that given in the above example to vary the consistency of the slurry and to regulate the setting time of the plaster in the completed bandage. The stirring time after the addition of the plaster of Paris likewise affects the setting time. Such matters, however, are within the province of the operators skilled in the art. For example, the above batch with 900 ml. of Elvacet 81A-900, stirred for fifteen minutes after adding the plaster of Paris, gave a bandage having a setting time of five to eight minutes. This bandage lost a negligible amount of plaster (less than 1%) when immersed in water, delivered from 94 to 96% of the plaster to the cast, and would not telescope until it had been soaked in water from 1% to 2 minutes. Within 3 to 5 seconds, however, the bandage will have soaked up

enough water for use. Thus, for all practical purposes, telescoping has been eliminated. Some idea may be had of the actual amount of adhesive used in this bandage when it is realized that 900 ml. of Elvacet 81A-900 weighs 2.15 lbs., the polyvinyl acetate solids content being about 1.18 lbs.

Another process which may be used to incorporate a non-swellable adhesive in a plaster of Paris bandage involves the use of ammonium borate to retard the setting of the plaster of Paris during the coating process. Ammonium borate, even in very small quantities, acts to retard the setting of plaster of Paris and it is particularly desirable for the purposes of this invention since, when it decomposes as the bandage is dried after coating, boric acid is left which has a negligible effect on the setting time of the plaster when the bandage subsequently is placed in use.

There follow several examples of batches or mixtures involving the foregoing process and which may be used to produce bandages according to the instant invention.

#### Example II

|                                                       | Pounds      |
|-------------------------------------------------------|-------------|
| Plaster of Paris                                      | 100         |
| Water                                                 | 50 to 100   |
| Copolymer of vinyl acetate and acrylic ester emulsion | 2 to 4      |
| Boric acid                                            | .5 to 2     |
| Aqua ammonia (29%)                                    | .685 to 2.8 |

#### Example III

|    |                            |             |
|----|----------------------------|-------------|
| 35 | Plaster of Paris           | 100         |
|    | Water                      | 50 to 100   |
|    | Polyvinyl acetate emulsion | 2.5 to 6    |
|    | Boric acid                 | .5 to 2     |
|    | Aqua ammonia (29%)         | .685 to 2.8 |

#### Example IV

|    |                                                         |             |
|----|---------------------------------------------------------|-------------|
| 35 | Plaster of Paris                                        | 100         |
|    | Water                                                   | 50 to 100   |
|    | Copolymer of vinyl acetate and methyl acrylate emulsion | 2.5 to 6    |
|    | Boric acid                                              | .5 to 2     |
|    | Aqua ammonia (29%)                                      | .685 to 2.8 |

The emulsion referred to in Example II is one made in this country by E. I. du Pont de Nemours and sold under the designation "TLF-223E." It contains 32% solids.

The polyvinyl acetate emulsion referred to in Example III is one made in this country by the Onyx Oil Company and sold under the designation A-101. It contains 25% solids.

The vinyl acetate methyl acrylate copolymer referred to in Example IV is made in this country by the Onyx Oil Company and sold under the designation A-2B. It contains 25% solids.

In the case of each of the above examples, the boric acid, aqua ammonia and water are mixed. The emulsion is dispersed therein and the plaster added. The mixture is stirred until there results a smooth slurry which is applied to a carrier of the usual type such as crinoline, gauze or other flexible fibrous material.

The coated carrier is dried, preferably by heat insufficient to bring the temperature of the coated carrier above 195° F., which is not sufficient to cause the adhesive to melt down to a continuous film, but which is so regulated that the hydrolysis of the ammonium borate (formed from the boric acid and aqua ammonia) is as complete as possible.

In general, the emulsions of water insoluble polymers to which reference has been made heretofore are prepared by dispersing in water the monomer of the material together with the dispersing agent and then polymerizing. Usually, the dispersing agent is a colloidal polyhydric agglutinant. Thus, in the polyvinyl acetate emulsion Elvacet 81A-900, the colloidal polyhydric agglutinant is polyvinyl alcohol, which is present to the extent of about 3% by weight. This emulsion, for stability, is buffered to a pH of between 4 and 7 by a suitable agent such as sodium acetate.

The invention has been described with reference to its preferred embodiments but other methods and materials within the invention's spirit will occur to those skilled in the art. For example, the hot water process in which no retardant is used but in which the water slurry is maintained around 95° C. may be used provided the non-swellable adhesive is in the form of an emulsion which is stable at such temperatures. It should be noted that substantially any non-swellable adhesive may be used provided it is in the form of an emulsion which is stable at the conditions under which the plaster of Paris slurry is made. The invention, therefore, is to be limited only by the prior art and the scope of the appended claims.

This application is a continuation-in-part of copending U. S. patent application, Serial No. 654,819, filed March 15, 1946, now abandoned.

What we claim is:

1. A plaster of Paris bandage comprising a flexible carrier and a coating of plaster of Paris thereon, the plaster of Paris being in the form of fine particles bonded to one another and to the flexible carrier by discrete particles of an adhesive which is non-swellable in water of the group consisting of high viscosity polyvinyl acetate, copolymers of vinyl acetate-acrylic ester, and copolymers of vinyl acetate-vinyl chloride, said adhesive being dispersed throughout the plaster of Paris coating, the adhesive being present in an amount within the range of from 0.1 to 2.5% based on the dry weight of plaster of Paris.

2. The method of preparing a plaster of Paris bandage which comprises making a water slurry of plaster of Paris in the presence of a sufficient amount of retardant of the group consisting of acetic acid and ammonium borate to prevent setting of the plaster, introducing an emulsion of a water insoluble vinyl acetate polymer into the slurry, coating a flexible carrier with the slurry and drying the carrier whereby there is left on the carrier plaster of Paris in the form of fine particles bonded to one another and to the flexible carrier by the insoluble vinyl acetate polymer in the form of discrete particles dispersed throughout the coating, adhesive being present in an amount within the range from 0.1 to 2.5% based on the dry weight of plaster of Paris.

3. A bandage according to claim 1 in which the adhesive is high viscosity polyvinyl acetate.

4. A bandage according to claim 1 in which the adhesive is a copolymer of vinyl acetate and acrylic ester.

5. A bandage according to claim 1 in which the adhesive is a copolymer of vinyl acetate and vinyl chloride.

6. A plaster of Paris bandage comprising a flex-

ible carrier and a coating of plaster of Paris thereon, the plaster of Paris being in the form of fine particles bonded to one another and to the flexible carrier by an adhesive which is dispersed throughout the plaster of Paris before coating said plaster of Paris on said carrier, by mixing an emulsion of said adhesive with a water slurry of said plaster of Paris in the presence of a sufficient amount of a retardant of the group consisting of acetic acid and ammonium borate to prevent setting of the plaster, said adhesive being non-swellable in water and present in an amount within the range of from 0.1 to 2.5% based on the dry weight of plaster of Paris.

7. A bandage according to claim 6 in which the adhesive is a high viscosity vinyl acetate polymer.

8. The method of preparing a plaster of Paris bandage which comprises making a water slurry of plaster of Paris in the presence of a sufficient amount of a retardant of the group consisting of acetic acid and ammonium borate to prevent setting of the plaster, introducing an emulsion of a water insoluble polyvinyl resin into the slurry, coating a flexible carrier with the slurry and drying the carrier whereby there is left on the carrier plaster of Paris in the form of fine particles bonded to one another and to the flexible carrier by the insoluble polyvinyl resin dispersed throughout the coating, said adhesive being present in amount within the range from 0.1 to 2.5% based on the dry weight of plaster of Paris.

9. A plaster of Paris bandage material comprising a flexible carrier and a coating of plaster of Paris thereon, the plaster of Paris being in the form of fine particles bonded to one another and to the flexible carrier by a nonwater-swellable adhesive which is dispersed throughout the plaster of Paris before coating said plaster of Paris on said carrier, by mixing an emulsion of said adhesive with said plaster of Paris to form a water slurry of plaster of Paris containing adhesive, said adhesive at the time the plaster of Paris is coated on said carrier being nonswellable in water and present in an amount within the range of from 0.1 to 2.5% based on the dry weight of plaster of Paris.

10. A bandage material according to claim 9 in which the adhesive is a water insoluble polyvinyl resin.

11. A bandage material according to claim 9 in which the adhesive is a water insoluble vinyl acetate polymer.

JAMES JOSEPH EBERL.  
ALVIN RICHARD INGRAM.

References Cited in the file of this patent

UNITED STATES PATENTS

| Number    | Name           | Date          |
|-----------|----------------|---------------|
| 2,152,670 | Shutte         | Apr. 4, 1939  |
| 2,218,710 | Herrmann       | Oct. 22, 1940 |
| 2,483,806 | Buckley et al. | Oct. 4, 1949  |

FOREIGN PATENTS

| Number  | Country       | Date          |
|---------|---------------|---------------|
| 368,421 | Italy         | Feb. 15, 1939 |
| 388,031 | Great Britain | Feb. 14, 1933 |

OTHER REFERENCES

Canadian Medical Association Journal for August 1945, pp. 170-1. Copy in Div. 55.